

# United States Patent Office

2,945,737

Patented July 19, 1960

1

2,945,737

## METHOD OF DEHAIRING HIDES

Thomas C. Thorstensen, Chelmsford, Mass., assignor to  
Tanners' Council of America, Inc., New York, N.Y.,  
a corporation of New York

No Drawing. Filed Apr. 25, 1957, Ser. No. 654,993

5 Claims. (Cl. 8—94.16)

This invention is concerned with the preparation of leather and is directed specifically to the problem of unhauling cattle hides, or dewoaled sheep or goatskins, preparatory to their conversion to leather. It aims to provide a process which gives much faster hair removal than conventional methods, without injury to the hide or to the hair which is removed, and with less disturbance of the hide substance than in the conventional processes. According to my invention, I treat the soaked hides or skins first with an aqueous alkaline solution of a strong reducing agent at a relatively low pH (not above 11.0 within a few minutes after the addition of the hides), maintain contact for a few hours, draw off the reducing agent and preferably wash the hides or skins, then treat the hides or skins for a few hours with an alkaline bath which is characterized by the presence of ammonium ions and a pH of at least 10 but below 12, to complete the loosening of the hair, and then remove the loosened and loosely attached hair from the hides or skins by conventional methods. Ordinary ambient temperatures (60 to 100° F.) are used throughout the process.

In the conventional tannery, hair removal is accomplished in the "beam-house." Cattle hides, or sheep or goat skins from which the wool has been removed leaving the shorter hairs, are dehaired for further processing using techniques which save the hair. In the standard processes, the hides are soaked for four to six days in a depilatory solution, consisting of an alkaline reducing agent and lime, which softens and loosens the hair, which is then removed in machines which scrape it from the skins and hides. The hair is washed and dried, and has an appreciable market value. However, some injury may be done to the skin in the process; and the long time required has been the source of considerable additional cost of operation.

Many attempts have been made to shorten the time required for the dehauling operation, and a number of processes have been suggested. But none of the methods have succeeded in getting the combination of shortened time, satisfactory hair removal, satisfactory hair recovery and satisfactory skin condition for leather manufacture.

According to my invention, I obtain all these desired objects by treating soaked hides or skins at ordinary ambient temperatures with an aqueous alkaline solution of a strong reducing agent, at a pH of below 11 for a period of a few hours, then preferably washing the hides or skins with water, then treating the skins for a few hours with an aqueous alkaline bath containing ammonium ions at a pH of 10 or more, but under 12, and then mechanically removing the loose and loosened hair from the hides or skins. Ordinary ambient temperatures are used throughout the process.

In the first bath, it is essential to use alkaline reducing agents which are strong enough to affect the S—S link in the cystine present in the older hair, and to reduce at least a portion of the cystine to cysteine, whereby the hydrolysis of the keratinous proteins of the hair follicles and epidermal layer can be accomplished by

2

aqueous alkali. I have found that the alkali metal sulfides and cyanides are most effective as reducing agents; the alkali metal sulfides and polysulfides, which are converted to sulfhydrates by the necessary pH adjustment, are just as effective but slightly less desirable economically; and the sulfites, bisulfites and hydrosulfites are all satisfactory, although a trifle slower in action. But sodium thiocyanate, for example, is not a powerful enough reducing agent to affect the S—S linkage in the cystine under the conditions necessary for preserving the hair and skin.

Generally, the reducing agent is present in the bath at a concentration of between 0.5 and 2.0% (about 2 to 10% based on hide weight). More reducing agent than 2% is generally wasted, while concentrations under 0.5% act so slowly that the contact time must be prolonged to such an extent that quality suffers.

The pH of this solution is held below 11.0 during the period of treatment since higher pH will cause deterioration in the quality of the recovered hair and substantial reduction in yield of saleable hair. In addition, there is some danger of attacking the skin itself. With some reducing agents, such as the cyanides, which contribute to raising the pH and which are rapidly used up with marked reduction of pH, the initial pH may be slightly over 11.0, since the pH drops so rapidly below 11.0 that no damage is done.

Enough bath is used to effectively cover the hides, and permit agitation of the hides in the solution. In most 30 plant equipment, the solution will run 3 to 5 times the hide weight, although this can vary widely.

The first treatment should continue for at least an hour, and a two hour treatment under agitation is most effective. Where convenient, the skins may be left in 35 the bath for longer periods, up to 12 hours or more, without real damage, due to the low pH.

The skins are preferably washed after the first treatment to minimize carryover of solution. The washing is not essential; but since carryover varies from batch to 40 batch, better control of the operation is obtained if the skins are washed to reduce the actual carryover of chemicals.

The second bath treatment serves to hydrolyze some 45 of the keratinous proteins of the hair and epidermis, so that the base comes out easily, but it is essential to control the action so that the hair is not destroyed. I obtain this desirable result by using an aqueous alkaline bath at a pH of at least 10.0 and below 12.0, the bath containing ammonium ions representing at least 0.15% 50 NH<sub>3</sub>, and preferably containing about 0.3% NH<sub>3</sub>. More ammonium ions can be used without injury, but are economically unsound.

The necessary pH may be obtained by buffering with a phosphate, or in any other desired manner. It is essential that the pH in this bath be at least 10, since hair loosening is too slow at lower pH's. At pH 12 or above, the tendency toward hair damage becomes marked and this is often accompanied by an actual decrease in the ease of hair removal. Hence, a pH of 12.0 or higher 55 should be avoided.

Preferably, the alkali treatment should be limited to about 2 hours, with good agitation. Poor agitation results in excessive hair loss locally; prolonged contact results in increasing hair damage with time, often accompanied by a decrease in the ease of hair removal.

60 The invention is exemplified by the following specific examples:

### Example 1.—Dehauling of cow hides

Four hides, weighing 200 pounds in the green salted 65 state, were washed in a wheel, trimmed, fleshed, and cut into two.

They were then placed in a paddle agitator containing

1,000 pounds of water at 90° F., in which was dissolved 12.5 pounds of sodium sulfhydrate. The pH of the solution was 9.5. The hides were paddled for a total of 2 hours, and then held 6 hours.

The stock was removed, and washed 5 minutes in water at 80° F. to flush off the first solution. The batch was then placed in a second bath consisting of

|                                                | Pounds |
|------------------------------------------------|--------|
| Water at 80° F.                                | 1,000  |
| Tech ammonium hydroxide (28% NH <sub>3</sub> ) | 10     |
| Trisodium phosphate                            | 20     |
| pH 11.6.                                       |        |

This batch was agitated for 2 hours, and the stock removed for unhairing. Unhairing was excellent; the hair yields were good, and the hair and skins were of excellent quality.

This example indicates the time latitude permissible in the first step.

*Example 2.—Unhairing of kip*

8 kip sides, weighing 100 pounds, were placed in a conventional tumbling mill and soaked overnight at 75° F. in a bath comprising

|                                   |  |
|-----------------------------------|--|
| 400 pounds water                  |  |
| 20 pounds urea                    |  |
| 2 pounds anhydrous sodium sulfite |  |
| pH 8.5.                           |  |

The batch was milled for an hour, and the skins were pulled and fleshed. The fleshed hides were returned to the mill, from which the soak liquor had been removed, and they were milled for an hour at 75° F. in a bath comprising

|                             |  |
|-----------------------------|--|
| 200 pounds water            |  |
| 3 pounds sodium sulfhydrate |  |

This solution was drained well and replaced by a solution consisting of

|                                              |  |
|----------------------------------------------|--|
| 200# water at 75° F.                         |  |
| 4# soda ash                                  |  |
| 0.4# caustic soda                            |  |
| 1/2# sodium sulfhydrate                      |  |
| 20# urea (to improve dispersing action)      |  |
| 4# ammonium hydroxide (28% NH <sub>3</sub> ) |  |
| pH 10.8.                                     |  |

The batch was milled 15 minutes, allowed to rest 2 hours, milled for a few minutes, and allowed to rest 1 1/2 hours. At this point (just short of 4 hours total) hair removal was excellent, the hides were of fine quality, and the hair was recoverable.

A few of the hides were left in the bath for observation, without stirring for another 4 hours. At this point, the hides were definitely swollen, and unhairing was no longer as satisfactory. This indicated clearly that the hydrolysis bath must not be allowed to act more than a few hours.

*Example 3.—Sodium sulfite unhairing*

2000 grams of green cattle hides were soaked overnight in water at 80° F., and then tumbled, with mild agitation, for two hours in a 1% solution of anhydrous sodium sulfite in 8000 grams of water at 80° F.; the batch was drained, rinsed, and tumbled for 2 hours in 8000 grams of water at 80° F. containing 1% concentrated ammonium hydroxide (28% NH<sub>3</sub>), 1% sodium carbonate and 0.1 caustic soda (pH 12.2). Unhairing was difficult because of the high pH. The recovered hair was of inferior quality.

*Example 4.—Sodium sulfite unhairing*

Example 3 was repeated, except the second bath contained 1% ammonium hydroxide and 2% trisodium phosphate (pH 11.6 to 11.8). This gave far superior unhairing to that obtained in Example 3, and illustrates,

with that example, the necessity for controlling the pH of the second bath.

*Example 5.—Potassium cyanide unhairing*

6 cowhide sides, weight 100# in the green salted state, and which had been soaked overnight in 400 pounds of a 1% aqueous solution of urea containing 0.2 pound sodium polysulfide, were washed in a paddle mill for 15 minutes with a 1% aqueous solution of ammonium hydroxide. The mill was drained, the stock trimmed and fleshed, and the stock was milled for 2 hours at 75° F. in a solution consisting of

|                            | Pounds |
|----------------------------|--------|
| Water                      | 100    |
| 29° Bé. ammonium hydroxide | 1      |
| Potassium cyanide          | 2 1/2  |

The water clinging to the hides immediately reduced the cyanide concentration to 1.5%; original pH was 10.31, dropping to 9.95 during the run, despite the addition of 2# ammonium hydroxide at the end of 15 minutes.

The cyanide solution was drained off into a lime pit, the stock was washed, and again milled for 2 hours at 75° F. after adding a solution of

|                                   | Pounds |
|-----------------------------------|--------|
| Water                             | 200    |
| Trisodium phosphate               | 2      |
| 29° Bé. ammonium hydroxide        | 4      |
| Original pH 11.67, final pH 11.0. |        |

*Example 6.—Potassium cyanide unhairing*

6 cowhide sides, weighing 101 pounds, in the green salted state, were soaked in conventional fashion to remove salt etc., and placed in a mill; and clinging water largely removed. A solution containing

|                                                           |  |
|-----------------------------------------------------------|--|
| 100 pounds water at 75° F.                                |  |
| 1 pound ammonium hydroxide; 29° Bé.                       |  |
| 2 1/2 pounds potassium cyanide                            |  |
| was added, and milling commenced. This solution was       |  |
| immediately reduced to 2.25% potassium cyanide by the     |  |
| water clinging to the hides; its initial pH of 11.7 was   |  |
| reduced in a few minutes to 11.0; was 10.9 at 15 minutes, |  |
| and 10.7 at the end of the two hour milling cycle.        |  |

The solution was withdrawn after 2 hours, and replaced by a solution containing

|                                      |  |
|--------------------------------------|--|
| 200 pounds water at 75° F.           |  |
| 4 pounds ammonium hydroxide; 29° Bé. |  |
| 5 pounds trisodium phosphate         |  |
| 1 pounds dimethylamine sulfate       |  |

The mill was run for five minutes, and then turned over 1 minute every fifteen minutes. At the end of two hours, the solution was drained. The pH ranged between 11.0 and 11.1 during the run.

Excellent unhairing was obtained.

It will be noted that in this example, the original pH in the first treating bath is somewhat above 11.0, but is rapidly reduced to below this figure, so that the actual treatment of the hides is almost all at a pH below 11.0.

I have shown but a few examples of the process, and it is obvious that these examples can be widely modified without departing from the scope of the invention which is defined in the claims.

I claim:

1. The process of dehairing cattle, sheep and goat hides in such fashion as to produce recoverable hair without damage to the hides, which comprises treating wet hides with a first, lime-free, bath comprising an aqueous alkaline solution of 2 to 10%, based on hide weight, of an alkali metal salt which has a reducing action strong enough to reduce the S—S linkage in cystine, for a period of at least an hour, the pH of the bath being maintained at a point not above 11.0 for substantially but not necessarily the entire treatment period;

removing the first bath, treating the hides for a few hours at ordinary ambient temperatures with a second bath comprising a lime-free aqueous alkaline solution containing ammonium ions representing at least 0.15% NH<sub>3</sub> and sodium ions, and maintained during the treatment at a pH of at least 10 and under 12.0, and then mechanically separating the loosened recoverable hair from the hides.

2. The process of claim 1, in which the reducing agent is selected from the group consisting of alkali metal sulf-  
hydrates and, cyanides.

3. The process of claim 1, in which the reducing agent is present in the first bath in an amount between 2 and 10% of hide weight.

4. The process of claim 1, in which the NH<sub>3</sub> concen-  
tration in the second bath is 0.3%.

5. The process of dehauling cattle, sheep and goat hides in such fashion as to produce recoverable hair without damage to the hides, which comprises treating wet hides with a first, lime-free bath comprising an aqueous alkaline solution of 2 to 10%, based on hide weight, of an alkali metal salt which has a reducing action strong enough to reduce the S—S linkage in cystine, for a period of at least an hour, the pH of the bath being maintained at a point not above 11.0 for substantially but not necessarily the entire treatment period, removing the first bath, wash-

ing the hides, then treating the hides for a few hours at ordinary ambient temperatures with a second bath comprising a lime-free aqueous alkaline solution containing ammonium ions representing at least 0.15% NH<sub>3</sub> and sodium ions, and maintained during the treatment at a pH of at least 10 and under 12.0, and then mechanically separating the loosened recoverable hair from the hides.

References Cited in the file of this patent

UNITED STATES PATENTS

2,487,558 Kamlet ----- Nov. 8, 1948  
2,775,504 Zalcman ----- Dec. 25, 1956

FOREIGN PATENTS

186,608 Great Britain ----- Jan. 21, 1924

OTHER REFERENCES

20 O'Flaherty: "Chem. and Tech. of Leather," Reinhold  
Publ. Co., N.Y., 1956, pp. 283, 282, 286 and 287.

"Progress in Leather Science," Br. Leather Manuf.  
Assoc., London, 1948 pp. 159, 161, 162, 164, 168, 169  
and 175-177.

25 Alderton: "The Leather World," 1944, vol. 36, pp.  
316-317, 396, 397, 462-464.

UNITED STATES PATENT OFFICE  
CERTIFICATE OF CORRECTION

Patent No. 2,945,737

July 19, 1960

Thomas C. Thorstensen

It is hereby certified that error appears in the printed specification of the above numbered patent requiring correction and that the said Letters Patent should read as corrected below.

Column 4, after line 28, insert the following sentence as line 29:

Excellent unhairing was obtained.

column 5, line 11, after "and" strike out the comma.

Signed and sealed this 31st day of January 1961.

(SEAL)

Attest:

KARL H. AXLINE

Attesting Officer

ROBERT C. WATSON  
Commissioner of Patents